

March 9, 1926.

1,576,141

J. N. SCHUMACHER

PLASTER BOARD

Filed Nov. 13, 1924

Fig. 1



Fig. 2



INVENTOR.

John N. Schumacher  
BY Westall and Wallace

ATTORNEYS.

## UNITED STATES PATENT OFFICE.

JOHN N. SCHUMACHER, OF LOS ANGELES, CALIFORNIA.

## PLASTER BOARD.

Application filed November 13, 1924. Serial No. 749,676.

*To all whom it may concern:*

Be it known that I, JOHN N. SCHUMACHER, a citizen of the United States, and resident of Los Angeles, county of Los Angeles, State 5 of California, have invented new and useful Improvements in Plaster Board, of which the following is a specification.

This invention relates to plaster board and the like comprising a cementitious body having a covering sheet of pliable material bonded thereto. It has been a desideratum in the manufacture of such articles to provide a method and material whereby the adhesion of the covering sheets and cementitious body is a maximum, and the board in its green state has characteristics permitting handling without damage. The time interval required for setting of the plaster body is an appreciable element in the production. Any method or means which will decrease the time element is desirable.

The primary objects of this invention are to provide an article of the character described and a method for producing the same which will decrease the time interval, maintain the quality of the article, and provide economy in manufacture.

These objects together with other objects and corresponding accomplishments are obtained by means of the embodiment of my invention illustrated in the accompanying drawing, in which:

Fig. 1 is a fragment of the length of plaster board constructed in accordance with my invention; and Fig. 2 is a transverse section through an edge thereof on an enlarged scale.

Referring more particularly to the drawing, a cementitious body 3 is shown interposed between covering sheets 4 and 5. The body 3 is preferably made of quick setting plaster. The covering sheets 4 and 5 are preferably of paper so treated as to be slowly permeable to moisture. With the paper 45 placed against the quick setting plaster, the resultant adhesion of the paper to the plas-

ter body would not reach the quality desired as the plaster would set before the moisture would permeate the covering sheets sufficiently to form a good bond. My invention 50 resides particularly in the treatment whereby a satisfactory adhesion is obtained. Quick setting plaster decreases the time element required for production of the board.

In order to overcome these objections, I 55 coat the inner face of each covering sheet with a layer of retarded plaster. This plaster will form a good bond with the body 3 and a satisfactory bond with the covering sheet. The layers of retarded plaster are 60 indicated by 6 and 7, and are in effect laminations. These laminations may be produced by passing the covering sheets in contact with plastic retarded plaster so that the latter will cling thereto, and then interposing the plaster board 3 therebetween in the manner well known in the art.

The plaster body 3 will set quickly producing a board stiff enough to handle without injury in a very short interval of time. 70 The laminations of retarded plaster board will assure a satisfactory adhesion between the covering sheets and the body.

What I claim is:

1. An article of the character described 75 comprising a quick setting cementitious body, a covering sheet of pliable material slowly permeable to moisture, and a lamination of retarded cementitious material binding said sheet and said body.

2. An article of the character described 80 comprising a body of quick setting plaster interposed between pliable sheets slowly permeable to moisture, and laminations of retarded plaster disposed on the outer faces 85 of said body and binding said sheets and body.

In witness that I claim the foregoing I have hereunto subscribed my name this 3rd day of November 1924.

JOHN N. SCHUMACHER.